

# United States Patent [19]

Ohaku et al.

[11] Patent Number: 4,728,592

[45] Date of Patent: Mar. 1, 1988

[54] ELECTROPHOTOCONDUCTOR WITH LIGHT-SENSITIVE LAYER CONTAINING ALPHA-TYPE TITANYL PHTHALOCYANINE

[75] Inventors: Kenichi Ohaku, Oyama; Hiroshi Nakano, Kitamoto; Masao Aizawa, Hasuda, all of Japan

[73] Assignee: Dainippon Ink and Chemicals, Inc., Tokyo, Japan

[21] Appl. No.: 886,496

[22] Filed: Jul. 17, 1986

[51] Int. Cl.<sup>4</sup> ..... G03G 5/06

[52] U.S. Cl. ..... 430/59; 430/76; 430/78

[58] Field of Search ..... 430/64, 76, 78, 59

## [56] References Cited

### U.S. PATENT DOCUMENTS

4,031,109 6/1977 Griffiths et al. ..... 430/76  
4,032,339 6/1977 Grushkin et al. ..... 430/1  
4,106,935 8/1978 Petruzzella ..... 430/64  
4,584,253 4/1986 Lin et al. ..... 430/64

### FOREIGN PATENT DOCUMENTS

0180930 5/1986 European Pat. Off. .

Primary Examiner—John L. Goodrow

Attorney, Agent, or Firm—Armstrong, Nikaido, Marmelstein & Kubovcik

## [57] ABSTRACT

An electrophotoconductor having a light-sensitive layer characterized in that a titanyl phthalocyanine is dispersed in a binder, said titanyl phthalocyanine having the structure represented by the general formula:



(wherein X<sub>1</sub>, X<sub>2</sub>, X<sub>3</sub> and X<sub>4</sub> each and independently represent Cl or Br; and k, l, m and n each and independently represent 0 or an integer of 1 to 4) and an alpha-type crystallographic form.

31 Claims, 9 Drawing Figures

FIG. 1



FIG. 2



FIG. 3



FIG. 4



FIG. 5



FIG. 6



FIG. 7



FIG. 8



FIG. 9



**ELECTROPHOTOCONDUCTOR WITH  
LIGHT-SENSITIVE LAYER CONTAINING  
ALPHA-TYPE TITANYL PHTHALOCYANINE**

**FIELD OF THE INVENTION**

**Background of the Invention**

The present invention relates to an electrophotoconductor and, more particularly, to one which is suitable for use in a printer such as a laser beam printer employing a semiconductor laser.

**Prior Art**

Since the discovery of the photoconductivity of phthalocyanine compounds in 1968, various studies have been conducted with respect to their use as photoconductive materials. With the recent advances in non-impact printing technology, active efforts are being made to develop laser beam printers which use semiconductor lasers for writing heads. Electrophotography with a laser beam printer starts with the formation of a uniform charged layer on a photoconductor by corona discharge, and after the charged photoconductor has been irradiated with a modulated laser beam in response to an input signal, a visible image is formed by toner development. This laser recording system has the advantages of improved image quality and a reduction in the complexity, size and cost of the printing system by virtue of the use of a semiconductor laser.

Most of the semiconductor lasers available today for stable operation have oscillation wavelengths in the near-infrared region ( $\lambda > 780$  nm). This means that photoconductors which are suitable for printing with such semiconductor lasers are required to have high sensitivity in the wavelength region longer than 780 nm. For practical purposes, sensitivities of 10 erg/cm<sup>2</sup> or less in terms of  $E^{\frac{1}{2}}$  are required, this being the exposure of monochromatic infrared radiation necessary to reduce the charge by half its initial value. While various photoconductive materials are known to exhibit high sensitivity at wavelengths longer than 780 nm, particular attention is being paid to phthalocyanine compounds.

Heretofore, electrophotoconductors have employed inorganic compounds such as selenium, tellurium, cadmium sulfide and zinc oxide, or organic compounds such as poly(N-vinylcarbazole) and bisazo pigments. However, none of these compounds have adequately high photosensitivity in the wavelength region longer than 780 nm. It has recently been reported that photoconductors using alloys containing selenium, tellurium or arsenic or dye-sensitized cadmium sulfide have high sensitivity in the wavelength region up to about 800 nm, but all of these compounds are highly toxic and social concern over environmental hazards has put the safety of these compounds into question. Photoconductors using amorphous silicon are also known and it is held that their sensitivity range can be extended to the longer wavelength region by selection of appropriate doping and production methods. But with the present state of the art, photoconductors using amorphous silicon are not available at low cost because the film of amorphous silicon cannot be deposited at a sufficiently fast rate to realize high-mass production. Among the phthalocya-

nine compound that have been reviewed and which have been shown to exhibit high sensitivity in the wavelength region longer than 780 nm are included X-type non-metallic phthalocyanine,  $\epsilon$ -type copper phthalocyanine, vanadyl phthalocyanine, etc.

With a view to attaining higher sensitivity, multi-layer photoconductors using a deposited phthalocyanine layer as a charge generation layer have been reviewed and in several cases, comparatively high sensitivities have been attained with phthalocyanine compounds having a metal of group IIIa or IV in the Periodic Table as the central metal.

However, the organic photoconductors of this type are costly because the formation of deposited layers required an expensive evacuation apparatus capable of producing very low ultimate pressures.

A different type of multi-layer photoconductors has also been reviewed; instead of being vacuum-evaporated, in this type phthalocyanine is dispersed in a resin to form a charge generation layer, on which is coated a charge transport layer. Photoconductors of this type use non-metallic phthalocyanine (U.S. Pat. No. 4,507,374) or indium phthalocyanine (U.S. Pat. No. 4,471,039) and both exhibit fairly high photosensitivity. However, the photoconductor using non-metallic phthalocyanine has the disadvantage that its sensitivity drops sharply in the wavelength region longer than 800 nm, and the one using indium phthalocyanine suffers from the disadvantage that the charge generation layer as a resin dispersion system cannot be formed on a commercial scale without sacrificing the sensitivity of the photoconductor.

**SUMMARY OF THE INVENTION**

The principal object, therefore, of the present invention is to eliminate the aforementioned defects of the prior art products and to provide an electrophotoconductor which exhibits high sensitivity over a broad wavelength range of 500-900 nm, especially in the wavelength region longer than 800 nm.

This object of the present invention can be attained by an electrophotoconductor which has a light-sensitive layer wherein a specified alpha-type titanyl phthalocyanine is dispersed in a binder.

**BRIEF DESCRIPTION OF THE DRAWINGS**

FIG. 1 is an X-ray diffraction pattern with Cu-K $\alpha$  for the alpha-type titanyl phthalocyanine used in the present invention;

FIGS. 2 to 5 are partial enlarged cross sections of electrophotoconductors produced in accordance with the present invention;

FIG. 6 is a graph showing the spectral sensitivities of the electrophotoconductors prepared in Examples 1 and 2;

FIG. 7 is a diagram showing the visible light absorption spectrum of the light-sensitive layer in the photoconductor prepared in Example 1;

FIG. 8 is an X-ray diffraction pattern for the light-sensitive coating formed in Example 1; and

FIG. 9 is an X-ray diffraction pattern for a beta-type titanyl phthalocyanine.

#### DETAILED DESCRIPTION OF THE INVENTION

The alpha-type titanyl phthalocyanine used in the present invention has the following general formula (I):



wherein  $X_1$ ,  $X_2$ ,  $X_3$  and  $X_4$  each and independently represents Cl or Br; and  $k$ ,  $l$ ,  $m$  and  $n$  each and independently represents 0 or an integer of 1 to 4.

Among the compounds of the general formula (I), those which are unsubstituted by any halogen of mono-halogen-substituted derivatives are particularly advantageous.

The alpha-titanyl phthalocyanine used in the present invention may be prepared, for example, by the following procedures: Titanium tetrachloride (or titanium tetrabromide) is reacted with phthalodinitrile in the solvent  $\alpha$ -chloronaphthalene to form dichlorotitanium phthalocyanine ( $TiCl_2Pc$ ) [for dibromotitanium phthalocyanine ( $TiBr_2Pc$ )]; it is then hydrolyzed with aqueous ammonia or any other appropriate hydrolyzing agent and the resulting product is treated with an electron-donating solvent such as 2-ethoxyethanol, diglyme, dioxane, tetrahydrofuran, N,N-dimethylformamide, N-methylpyrrolidone, pyridine or morpholine.

An X-ray diffraction pattern for the so prepared alpha-type titanyl phthalocyanine [ $k=1=m=n=0$  in the general formula (I)] with Cu-K $\alpha$  radiation is shown in FIG. 1, from which one can see that this alpha-type titanyl phthalocyanine has characteristic peaks at Bragg angles ( $2\theta$ ) of 7.6, 10.2, 12.6, 13.2, 15.1, 16.2, 17.2, 18.3, 22.5, 24.2, 25.3, 28.6, 29.3 and 31.5 (inclusive of errors within the range of  $\pm 0.2$  degrees).

The other alpha-type titanyl phthalocyanines which can be used in the present invention differ from the compound shown above with respect to the halogen atom as a substituent, the position of substituent, or the number of substituents, but all of them provide X-ray diffraction pattern having the same characteristic peaks as indicated in FIG. 1.

The titanyl phthalocyanine used in the present invention is preferably milled to adequately fine particles with milling machines, such as ball mills, sand mills or attritors. Milling operation may be performed in the presence of common milling media such as glass beads, steel beads or alumina beads. If necessary, milling aids

such as sodium chloride or sodium bicarbonate may be employed. If dispersion media are used during the milling operation, those which are liquid at the milling temperature are preferably used. Illustrative dispersion media are such solvents as 2-ethoxyethanol, diglyme, dioxane, tetrahydrofuran, N,N-dimethylformamide, N-methylpyrrolidone, pyridine, morpholine, polyethylene glycol and the like.

10 Any of the resins which are commonly employed as binders in electrophotoconductors may be used as binders in the present invention, and advantageous examples include a phenol resin, urea resin, melamine resin, epoxy resin, silicone resin, vinylchloride-vinyl acetate copolymer, butyral resin, xylene resin, urethane resin, acrylic resin, polycarbonate resin, polyacrylate resin, saturated polyester resin, phenoxy resin, etc.

The electrophotoconductor of the present invention 20 may assume various structures as shown in FIGS. 2 to 5. The photoconductor shown in FIG. 2 consists of an electrically conductive support (hereinafter referred to as a conductive support) (1) which is overlaid with a light-sensitive layer (2a) wherein the alpha-type titanyl phthalocyanine (3) is dispersed in a binder (4). The photoconductor shown in FIG. 3 consists of a conductive support (1) which is overlaid with a light-sensitive layer (2b) wherein the alpha-type titanyl phthalocyanine (3) is dispersed in a charge transport medium (5) comprised of a charge transport material and a binder. The photoconductor shown in FIG. 4 (or FIG. 5) consists of a conductive support (1) which is overlaid with a light-sensitive layer (2c) (or 2d) composed of a charge generation layer (6) having the alpha-type titanyl phthalocyanine (3) dispersed in a binder (4) and a charge transport layer (7) comprised of a charge transport material and a binder.

30 In the photoconductor shown in FIG. 2, the alpha-type titanyl phthalocyanine (3) serves to both generate and transport charges to cause the necessary light decay. In the photoconductor shown in FIG. 3, the charge 35 transport material combines with the binder to form the charge transport medium (5), with the alpha-type phthalocyanine (3) serving as a charge generation material. The charge transport medium (5) has the capability of accepting and transporting the charge generated 45 from the titanyl phthalocyanine. Therefore, in the photoconductor of FIG. 3, the titanyl phthalocyanine is responsible for the production of the charge carriers necessary to cause light decay while the so produced charge are transported principally by the charge transport medium (5). In the photoconductors shown in FIGS. 4 and 5, the alpha-type titanyl phthalocyanine (3) present in the charge generation layer (6) serves to 50 generate charges, while are injected into and transported through the charge transport layer (7).

The photoconductor of FIG. 2 may be prepared by dispersing the titanyl phthalocyanine in a solution of the binder, coating the dispersion onto a conductive support, and then drying the web. The photoconductor of FIG. 3 may be prepared by dispersing the titanyl phthalocyanine in a solution of the charge transport material and the binder, coating the dispersion onto a conductive

support, and then drying the web. The photoconductor of FIG. 4 may be prepared by dispersing the titanyl phthalocyanine in a binder solution, coating the dispersion onto a conductive support, drying the coated layer, then coating a solution of the charge transport material and binder in a suitable solvent, and finally drying the web. The photoconductor of FIG. 5 may be prepared by dissolving the charge transport material and binder in a suitable solvent, coating the solution onto a conductive support, drying the coated layer, then coating a dispersion of the titanyl phthalocyanine in a binder solution, and finally drying the web. Coating operation is typically conducted by roll coating, wire bar coating, or doctor blade coating.

The light-sensitive layer has a thickness ranging from 3 to 50  $\mu\text{m}$ , preferably from 5 to 20  $\mu\text{m}$ , in the case of the photoconductors shown in FIGS. 2 and 3. If the light-sensitive layer has a dual structure as in the case of the photoconductors shown in FIGS. 4 and 5, the charge generation layer has a thickness of 5  $\mu\text{m}$  or below, preferably between 0.01 and 2  $\mu\text{m}$ , and the charge transport layer has a thickness ranging from 3 to 50  $\mu\text{m}$ , preferably from 5 to 20  $\mu\text{m}$ .

The alpha-type titanyl phthalocyanine is present in the light-sensitive layer of the electrophotoconductor of the present invention in an amount ranging from 0.05 to 90%, preferably from 5 to 50%, of the weight of the light-sensitive layer.

In order to attain an even higher sensitivity, the electrophotoconductor of the present invention may optionally contain a charge transport material and/or a charge generation material in the light-sensitive layer together with the alpha-type titanyl phthalocyanine. In this case, 100 parts by weight of the alpha-type titanyl phthalocyanine is preferably combined with 10-1,000 parts by weight of the charge transport material and/or 1 to 500 parts by weight of the charge generation material. In a more preferable case, 100 parts by weight of the alpha-type titanyl phthalocyanine is combined with 100-500 parts by weight of the charge transport material and 5-50 parts by weight of the charge generation material.

Examples of the charge transport material which may be used in the present invention include indoline, quinoline, triphenylamine compounds, etc. Illustrative charge generation materials are perylene and bisazo compounds. Needless to say, these charge generation materials are also capable of charge transport.

Usable indoline compounds include those which are represented by the following general formulae:



(wherein R<sub>1</sub> is an optionally substituted alkyl, aralkyl or aryl group; R<sub>2</sub> and R<sub>3</sub> each independently represents a hydrogen atom, a halogen atom, or an optionally substituted alkyl, aralkyl or aryl group; R<sub>4</sub> is a hydrogen

atom, a halogen atom or an optionally substituted alkyl or aralkyl group; R<sub>5</sub> and R<sub>6</sub> each independently represents an optionally substituted alkyl, aralkyl or aryl group, provided that R<sub>5</sub> and R<sub>6</sub> may combine with each other to form a ring); and



(wherein A is an optionally substituted aromatic hydrocarbon group or aromatic heterocyclic group; and R<sub>1</sub>' and R<sub>2</sub>' each independently represents a hydrogen atom, a halogen atom, or an optionally substituted alkyl, aralkyl or aryl group).

Advantageous examples of the indoline compound are listed in Table 1 below.

TABLE 1

Indoline Compound (1)

| No. | Structure of A | -R <sub>1</sub> ' | -R <sub>2</sub> ' |
|-----|----------------|-------------------|-------------------|
| T-1 |                | -H                | -H                |
| T-2 |                | -H                | -H                |
| T-3 |                | -H                | -H                |
| T-4 |                | -H                | -H                |
| T-5 |                | -H                | -H                |

TABLE 1-continued

|      |                                                                                     |                  |                  |    |
|------|-------------------------------------------------------------------------------------|------------------|------------------|----|
| T-6  |    | -H               | -H               |    |
| T-7  |    | -H               | -H               | 10 |
| T-8  |    | -H               | -H               | 15 |
| T-9  |    | -H               | -H               | 20 |
| T-10 |    | -CH <sub>3</sub> | -H               |    |
| T-11 |  | -H               | -H               |    |
| T-12 |  | -H               | -CH <sub>3</sub> | 45 |
| T-13 |  | -CH <sub>3</sub> | -CH <sub>3</sub> | 50 |
| T-14 |  | -CH <sub>3</sub> | -H               |    |
| T-15 |  | -H               | -H               |    |

TABLE 1-continued

|      |                                                                                      |                                                                                      |                  |    |
|------|--------------------------------------------------------------------------------------|--------------------------------------------------------------------------------------|------------------|----|
| T-16 |    | -CH <sub>3</sub>                                                                     | -H               |    |
| T-17 |    | -CH <sub>3</sub>                                                                     | -H               |    |
| T-18 |    | -CH <sub>3</sub>                                                                     | -H               |    |
| T-19 |   | -CH <sub>3</sub>                                                                     | -H               |    |
|      | Indoline Compound (2)                                                                |                                                                                      |                  |    |
| 40   |  |                                                                                      |                  |    |
| 45   | No. Structure of A' -R <sub>1</sub> -R <sub>2</sub>                                  |                                                                                      |                  |    |
| 50   | T-20                                                                                 |  | -CH <sub>3</sub> | -H |
| 55   |                                                                                      |  |                  |    |
| 60   | T-21                                                                                 |  | -CH <sub>3</sub> | -H |
| 65   |                                                                                      |  |                  |    |

TABLE 1-continued

|      |  |       |      |    |
|------|--|-------|------|----|
| T-22 |  | -C2H5 | -H   | 5  |
| T-23 |  | -C2H5 | -H   | 10 |
| T-24 |  | -C2H5 | -H   | 15 |
| T-25 |  | -C2H5 | -H   | 20 |
| T-26 |  | -CH3  | -CH3 | 25 |
| T-27 |  | -CH3  | -CH3 | 30 |
| T-28 |  | -CH3  |      | 35 |

Illustrative quinoline compounds are those which are represented by the following general formula:



15 (wherein B is an optionally substituted aromatic hydrocarbon group or aromatic heterocyclic group; R<sub>1</sub>''', R<sub>2</sub>''' and R<sub>3</sub> each independently represents a hydrogen atom, a halogen atom or an optionally substituted alkyl, aralkyl or aryl group). Advantageous examples of the quinoline compounds are listed in Table 2 below.

TABLE 2

Quinoline Compound (1)

| No.  | Structure of B | -R <sub>1</sub> ''' | -R <sub>2</sub> ''' |
|------|----------------|---------------------|---------------------|
| T-29 |                | -H                  | -H                  |
| 40   |                |                     |                     |
| T-30 |                | -H                  | -H                  |
| 45   |                |                     |                     |
| T-31 |                | -H                  | -H                  |
| 50   |                |                     |                     |
| T-32 |                | -H                  | -H                  |
| 55   |                |                     |                     |
| T-33 |                | -H                  | -H                  |
| 60   |                |                     |                     |
| T-34 |                | -H                  | -H                  |
| 65   |                |                     |                     |

TABLE 2-continued

**Quinoline Compound (1)**

| No.  | Structure of B | $-R_1''$ | $-R_2''$ |
|------|----------------|----------|----------|
| T-35 |                | $-H$     | $-H$     |
| T-36 |                | $-H$     | $-H$     |
| T-37 |                | $-H$     | $-H$     |
| T-38 |                | $-CH_3$  | $-H$     |
| T-39 |                | $-H$     | $-H$     |
| T-40 |                | $-H$     | $-CH_3$  |
| T-41 |                | $-CH_3$  | $-CH_3$  |
| T-42 |                | $-CH_3$  | $-H$     |
| T-43 |                | $-H$     | $-H$     |

TABLE 2-continued

**Quinoline Compound (1)**

5

$$\begin{array}{c}
 \text{B}-\text{C}=\text{N}-\text{N} \\
 | \quad \backslash \quad / \\
 \text{H} \quad \text{HC} \quad \text{CH}_2 \\
 \quad \quad | \quad | \\
 \quad \quad \text{R}_1'' \quad \text{R}_2'' \\
 \end{array}$$

10

No.

15 T-44

Structure of B

-R<sub>1</sub>''

-R<sub>2</sub>''

-CH<sub>3</sub>

-H

20

25 T-45

-CH<sub>3</sub>

-H

30

35 Illustrative triphenylamine compounds are those which are represented by the following general formula:



(wherein Ar<sub>1</sub>, Ar<sub>2</sub> and Ar<sub>3</sub> each independently represents a substituted or unsubstituted aromatic hydrocarbon group or a substituted or unsubstituted aromatic heterocyclic group). Advantageous examples of the triphenylamine compound are listed in Table 3 below.

TABLE 3

**Triphenylamine Compound**

55

$$\begin{array}{c}
 \text{Ar}_1 \quad \text{Ar}_2 \\
 | \quad \quad | \\
 \text{N} \\
 | \\
 \text{Ar}_3
 \end{array}$$

| No.  | —Ar <sub>1</sub>                                                                     | —Ar <sub>2</sub>                                                                      | —Ar <sub>3</sub>                                                                      |
|------|--------------------------------------------------------------------------------------|---------------------------------------------------------------------------------------|---------------------------------------------------------------------------------------|
| T-46 |  |  |  |
| T-47 |  |  |  |

Other well known charge transport materials may also be employed and they include derivatives of such heterocyclic compounds as pyrazole, pyrazoline, oxadiazole, thiazole, imidazole, etc.; hydrazone derivatives; triphenylmethane derivatives; and poly-N-vinylcarbazole and derivatives thereof.

Any of the bisazo compounds commonly used in electrophotographic photoconductors may be used in the present invention, and they include:

(1) Compounds of the general formula:



(wherein — A'' — is a divalent conjugate organic group; and — B'' — is a monovalent organic group);

(2) Compounds of the general formula:



(wherein — A'' — is a divalent conjugate organic group); and

(3) Compounds of the general formula:



5

10

30

35

(wherein — A'' — is a divalent conjugate organic group; and — B'' — is a monovalent organic group).

Advantageous examples of the bisazo compound which is suitable for use in the present invention are listed in Table 4 below.

TABLE 4

Bisazo Compound (1)



| No. | Structure of — A'' — |
|-----|----------------------|
| P-1 |                      |
| P-2 |                      |

TABLE 4-continued

P-3



P-4



P-5



P-6



P-7



P-8



P-9



P-10



P-11



P-13



P-14



P-15



P-16



TABLE 4-continued

P-17



P-18



P-19



P-20



P-21



P-22



P-23



Bisazo Compound (2)

P-12



Bisazo Compound (3)



No.

Structure of  $-\text{A}''-$  $-\text{X}$

TABLE 4-continued

P-24



-H

P-25



-Cl

P-26



-Cl

P-27



-H

P-28



-H

P-29



-H

P-30



-H

P-31



-H

P-32



-H

P-33



-H

P-34



-H

TABLE 4-continued

P-35



-H

P-36



-H

Bisazo Compound (4)



No.

Structure of -A''-

P-37



P-38



P-39



P-40



Bisazo Compound (5)



No.

Structure of -A''-

P-41



P-42



TABLE 4-continued

P-43



P-44



Bisazo Compound (6)



No.

Structure of  $(B'')$  —

—Y

—Cl

P-45



—Cl

P-46



—Cl

P-47



—Cl

P-48



—Cl

P-49



—Cl

P-50



—Cl

P-51



—Cl

P-52



—Cl

TABLE 4-continued

|      |                                                                                     |     |
|------|-------------------------------------------------------------------------------------|-----|
| P-53 |    | —Cl |
| P-54 |    | —Cl |
| P-55 |    | —Cl |
| P-56 |    | —Cl |
| P-57 |    | —Cl |
| P-58 |   | —Cl |
| P-59 |  | —Cl |
| P-60 |  | —Cl |
| P-61 |  | —Cl |
| P-62 |  | —Cl |
| P-63 |  | —Cl |
| P-64 |  | —Cl |

TABLE 4-continued

P-65



-Cl

P-66



-Cl

P-67



-Cl

P-68



-Cl

P-69



-Cl

P-70



-Cl

P-71



-Cl

P-72



-Cl

P-73



-Cl

TABLE 4-continued

P-74



-Cl

P-75



-Cl

P-76



-Cl

P-77



-CH3

P-78



-CH3

P-79



-CH3

P-80



-CH3

P-81



-CH3

P-82



-OCH3

P-83



-OCH3

TABLE 4-continued

P-84

-OCH<sub>3</sub>

P-85

-OCH<sub>3</sub>

P-86

-OCH<sub>3</sub>

P-87

-NO<sub>2</sub>

P-88

-NO<sub>2</sub>

P-89

-NO<sub>2</sub>

P-90

-NO<sub>2</sub>

P-91

-NO<sub>2</sub>

P-92



-H

TABLE 4-continued

P-93



-H

P-94



-Br

A perylene compound may be used as a charge generation material together with the titanyl phthalocyanine in the present invention and examples of usable perylene compounds are represented by the following general formula:



15

20

25

(wherein R<sub>1'''</sub> and R<sub>2'''</sub> each independently represents a hydrogen atom or a substituted or unsubstituted alkyl, aryl, alkylaryl or amino group).

Advantageous examples of the perylene compounds are listed in Table 5 below.

30

35

TABLE 5

Perylene Compound (1)



40

45

| No.   | -R <sub>1'''</sub> and -R <sub>2'''</sub>          |    |
|-------|----------------------------------------------------|----|
| P-95  | -NH <sub>2</sub>                                   |    |
| P-96  | -H                                                 |    |
| P-97  | -CH <sub>3</sub>                                   |    |
| P-98  | -CH <sub>2</sub> CH <sub>3</sub>                   |    |
| P-99  | -(CH <sub>2</sub> ) <sub>2</sub> CH <sub>3</sub>   |    |
| P-100 | -(CH <sub>2</sub> ) <sub>3</sub> CH <sub>3</sub>   |    |
| P-101 | -CH <sub>2</sub> CH <sub>2</sub> OH                |    |
| P-102 | -(CH <sub>2</sub> ) <sub>3</sub> -OCH <sub>3</sub> |    |
| P-103 |                                                    | 55 |

P-104



P-104



60

65

TABLE 5-continued

P-105



P-106



P-107



P-108



P-109



P-110



P-111



P-112



P-113



P-114



TABLE 5-continued

P-115



P-116



P-117



Perylene Compound (2)

P-118



The conductive support for the photoconductor of the present invention may be a metal (e.g. aluminum) plate or foil, a plastic film on which the vapor of a metal (e.g. aluminum) is deposited, or paper which has been rendered conductive.

If necessary, the electrophotoconductor of the present invention may have an adhesive layer or a barrier layer provided between the conductive support and the light-sensitive layer. An adhesive or barrier layer may be formed of a polyamide, nitrocellulose, casein or poly(vinyl alcohol), and its thickness is desirable not greater than 1  $\mu\text{m}$ .

The following examples are provided for the purpose of further illustrating the present invention. It should however be understood that various modifications may be made to the following examples without departing from the spirit and scope of the invention.

The compound numbers of the charge transport materials (i.e., indoline, quinoline and triphenylamine compounds) used in the following examples are indicated in Tables 1 to 3, while the compound numbers of the charge generation materials used in the same examples are noted in Tables 4 and 5 (i.e., bisazo and perylene compounds).

In the examples, all parts are on a weight basis unless otherwise specified.

#### EXAMPLE 1

##### (I) Preparation of Alpha-Type Titanyl Phthalocyanine

Titanium tetrachloride (18 g) and phthalodinitrile (40 g) were agitated in  $\alpha$ -chloronaphthalene (500 ml) at 240°-250° C. under a nitrogen stream. After completion of the reaction, the product dichlorotitanium phthalocyanine was recovered by filtration. The recovered dichlorotitanium phthalocyanine was heated under reflux for 1 hour together with concentrated aqueous ammonia (300 ml) and pyridine (300 ml) so as to obtain the end compound,  $\alpha$ -type titanyl phthalocyanine (18

g). This compound was thoroughly washed in a Soxhlet extractor first with N,N-dimethylformamide, then with acetone.

5 An X-ray diffraction pattern for the  $\alpha$ -type titanyl phthalocyanine thus obtained with Cu-K $\alpha$  radiation is shown in FIG. 1.

##### (II) Preparation of Electrophotoconductor

10 The  $\alpha$ -type titanyl phthalocyanine prepared in (I) was milled in a ball mill for 64 hours with alumina beads being used as a milling medium. On part of the fine particles of  $\alpha$ -type titanyl phthalocyanine, 6 parts of a saturated polyester resin (Vylon 200 by Toyobo Co., Ltd.) and 36 parts of a 4:6 liquid mixture of 1,1,2-trichloroethane/dichloromethane were mixed in a paint shaker for 2 hours with glass beads being used as a mixing medium. The resulting dispersion was applied to 15 an aluminum plate with a wire bar coater to form a light-sensitive layer having a dry thickness of 10  $\mu\text{m}$ .

The so prepared single-layer electrophotoconductor was subjected to a sensitivity test with a Paper Analyzer 20 SP-428 of Kawaguchi Electric Works Co., Ltd. by the following procedures: the photoconductor was charged to a positive voltage of 6 kV by corona discharge in the dark and the initial potential ( $V_0$ ) was measured; the charged photoconductor was then left in the dark for 10 25 seconds and the surface potential retention ( $V_{10}/V_0$  [%]) was measured; the photoreceptor was then exposed under a tungsten lamp for a surface illumination of 5 lux, and the photosensitivity  $E^{\frac{1}{2}}$  (or  $E^{1/5}$ ), or the exposure required for the surface potential to drop to 30 half (or one-fifth) of the initial value, was measured; in a similar manner, the surface potential retained after 15 35 seconds of exposure was measured;  $E^{\frac{1}{2}}$  and  $E^{1/5}$  values were also measured by illuminating the photoreceptor with monochromatic light at 830 nm (intensity, 10 40 mW/m<sup>2</sup>).

The spectral sensitivity of the photoreceptor is shown 45 in FIG. 6, from which one can see that over the broad range of 520 to 900 nm it exhibited sensitivities higher than  $E^{\frac{1}{2}}=0.1 \text{ cm}^2/\text{erg}$  ( $E^{\frac{1}{2}}=10 \text{ erg}/\text{cm}^2$ ) which is the value required for commercially acceptable photoconductors to be used with a laser printer.

A coating solution of light-sensitive material was 50 prepared as in Example 1 and applied to a transparent PET film. The visible light absorption spectrum of the obtained light-sensitive layer is shown in FIG. 7, with absorption maxima occurring at 650 nm and 830 nm. An 55 X-ray diffraction pattern for the same layer is shown in FIG. 8.

#### EXAMPLE 2

Three parts of the fine particles of  $\alpha$ -type titanyl phthalocyanine which were obtained as in Example 1, 1 60 part of a saturated polyester resin (Vylon 200) and 210 parts of chloroform were mixed in a ball mill for 18 hours with alumina beads being used as a mixing medium. The resulting dispersion was coated with a wire bar onto a polyester film having a vapor-deposited aluminum layer, so as to form a charge generation layer 65 having a dry thickness of 0.3  $\mu\text{m}$ .

A solution wherein 5 parts of a charge transport material (No. T-10) and 5 parts of a polycarbonate resin (Panlite-1250 by Teijin Chemicals Ltd.) was dissolved

The characteristics of the photoconductors prepared in Examples 1 to 3 and Comparative Examples 1 and 2 are summarized in Table 6 below.

TABLE 6

| Run No.     | V <sub>0</sub> (V) | V <sub>10</sub> /V <sub>0</sub> (%) | Illumination by tungsten lamp |                   |                     | Exposure to light at 830 nm  |                              |
|-------------|--------------------|-------------------------------------|-------------------------------|-------------------|---------------------|------------------------------|------------------------------|
|             |                    |                                     | E 1/2 (lux · sec)             | E 1/5 (lux · sec) | V <sub>15</sub> (V) | E 1/2 (erg/cm <sup>2</sup> ) | E 1/5 (erg/cm <sup>2</sup> ) |
| Example 1   | (+)-600            | 86.0                                | 0.7                           | 0.9               | 8                   | 3.6                          | 3.9                          |
| Example 2   | (-)-580            | 76.0                                | 0.8                           | 1.8               | 5                   | 2.7                          | 5.1                          |
| Example 3   | (+)-500            | 65.0                                | 1.4                           | 3.3               | 15                  | 6.5                          | —                            |
| Comparative | (+)-160            | 54.0                                | 4.4                           | not available     | 30                  | —                            | —                            |
| Example 1   |                    |                                     |                               |                   |                     |                              |                              |
| Comparative | (-)-390            | 60.3                                | 2.0                           | 5.6               | 8                   | 8.0                          | 22.4                         |
| Example 2   |                    |                                     |                               |                   |                     |                              |                              |

in 65 parts of chloroform was coated onto the charge generation layer with a wire bar, so as to form a charge transport layer having a dry thickness of 10  $\mu\text{m}$ .

The characteristics of the so prepared multilayer electrophotoconductor were evaluated as in Example 1 except that V<sub>0</sub> was measured with the photoconductor being charged to a negative voltage of 6 kV by corona discharge.

### EXAMPLE 3

A solution of 8 parts of a charge transport material (No. T-10) and 8 parts of a polyarylate resin (U-100 by Union Carbide Corporation) in 92 parts of dioxane was applied to form a layer having a dry thickness of 10  $\mu\text{m}$ . Three parts of the fine particles of  $\alpha$ -type titanyl phthalocyanine which were prepared as in Example 1, 1 part of a charge generation layer (No. P-53), 6 parts of a charge transport material (No. T-10), 15 parts of a polyarylate resin (U-100) and 150 parts of chloroform were mixed in a paint shaker and the resulting dispersion was applied to the charge transport layer, so as to form a charge generation layer having a dry thickness of 5  $\mu\text{m}$ . By these procedures, a multi-layer electrophotoconductor was obtained.

### COMPARATIVE EXAMPLE 1

Alpha-type titanyl phthalocyanine was prepared as in Example 1(I) and recrystallized from  $\alpha$ -chloronaphthalene. By further purification, beta-type titanyl phthalocyanine was obtained which had characteristic peaks at Bragg angles (2 $\theta$ ) of 7.4, 9.2, 10.3, 13.0, 14.9, 15.3, 15.9, 18.6, 20.6, 23.2, 25.5, 26.2, 27.0 and 32.7. An X-ray diffraction pattern for this beta-type titanyl phthalocyanine is shown in FIG. 9. A single-layer electrophotoconductor was prepared as in Example 1 except that the  $\alpha$ -type titanyl phthalocyanine was replaced by the above-prepared  $\beta$ -type titanyl phthalocyanine. The characteristics of the photoconductor were evaluated as in Example 1.

### COMPARATIVE EXAMPLE 2

A multi-layer electrophotoconductor was prepared as in Example 2 except that the  $\alpha$ -type titanyl phthalocyanine was replaced by the  $\beta$ -type titanyl phthalocyanine prepared in Comparative Example 1. The characteristics of the photoconductor were evaluated as in Example 1.

20

### EXAMPLES 4 TO 7

Three parts of the fine particles of titanyl phthalocyanine which were prepared as in Example 1, 1 part of a saturated polyester resin (Vylon 200) and 210 parts of one of the solvents shown in Table 7 were mixed in a ball mill for 18 hours with alumina beads being used as a mixing medium. The resulting dispersion was coated with a wire bar onto a polyester film having a vapor-deposited aluminum layer, so as to form a charge generation layer having a dry thickness of 0.3  $\mu\text{m}$ . Subsequently, a multilayer electrophotoconductor was prepared as in Example 2. Additional photoconductors were obtained by the same procedures. Each of the photoconductors was illuminated by light at 830 nm (intensity, 10 mW/m<sup>2</sup>) and its sensitivity (E 1/5) was measured. The results are shown in Table 7.

TABLE 7

| Example No. | Solvent                                        | E 1/5 (erg/cm <sup>2</sup> ) |
|-------------|------------------------------------------------|------------------------------|
| 4           | toluene                                        | 5.1                          |
| 5           | dioxane                                        | 5.1                          |
| 6           | tetrahydrofuran                                | 4.0                          |
| 7           | methylene chloride/1,2,2-trichloroethane (6/4) | 5.1                          |

### EXAMPLES 8 TO 15

Additional photoconductors were fabricated as in Example 2 except that the charge transport material (No. T-10) was replaced by one of the materials shown in Table 8. Each of the photoconductors thus fabricated was irradiated by light at 830 nm (intensity, 10 mW/m<sup>2</sup>) and its sensitivity (E 1/5) was measured. The results are shown in Table 8.

TABLE 8

| Example No. | Charge transport material No. | E 1/5 (erg/cm <sup>2</sup> ) |
|-------------|-------------------------------|------------------------------|
| 8           | T-9                           | 20.0                         |
| 9           | T-16                          | 5.1                          |
| 10          | T-17                          | 4.0                          |
| 11          | T-19                          | 4.4                          |
| 12          | T-24                          | 20                           |
| 13          | T-38                          | 4.4                          |
| 14          | T-41                          | 4.6                          |
| 15          | T-47                          | 8.0                          |

60

65

## EXAMPLE 16 TO 21

Three parts of the fine particles of  $\alpha$ -type titanyl phthalocyanine which were prepared as in Example 1, 1 5 part of a saturated polyester resin (Vylon 200), 210 parts of chloroform, and 0.9 parts of one of the charge generation materials listed in Table 9 were mixed in a ball mill for 18 hours with alumina beads being used as a mixing 10 medium. The resulting dispersion was coated with a wire bar onto a polyester film having a vapor-deposited aluminum layer, so as to form a charge generation layer having a dry thickness of 0.3  $\mu$ m. Subsequently, multi-layer electrophotoconductors were prepared as in Example 2. The so-prepared photoconductors had the characteristics summarized in Table 9.

TABLE 9

| Example No. | Charge generation material No. | $V_0$ (V) | $V_{10}/V_0$ (%) | Illumination by light at 830 nm<br>E 1/5 (erg/cm <sup>2</sup> ) |
|-------------|--------------------------------|-----------|------------------|-----------------------------------------------------------------|
| 16          | P-4                            | 640       | 82               | 5.2                                                             |
| 17          | P-17                           | 650       | 82               | 5.2                                                             |
| 18          | P-37                           | 665       | 84               | 5.4                                                             |
| 19          | P-47                           | 620       | 80               | 5.2                                                             |
| 20          | P-53                           | 650       | 82               | 5.4                                                             |
| 21          | P-104                          | 610       | 78               | 5.2                                                             |

The electrophotoconductor of the present invention 35 has a light-sensitive layer wherein the alpha-type titanyl phthalocyanine specified hereinabove is dispersed in a binder, and it has high sensitivity over a broad wavelength region of 500 to 900 nm. The photoconductor of 40 the present invention will provide particularly good results when it is used with a laser beam printer or an LED printer employing a light source having wavelengths within the range of 700-900 nm.

The application of the electrophotoconductor of the present invention is not limited to printing with laser beam printers; it can also be applied to various other optical recording devices employing light sources such as semiconductor laser operating at wavelengths longer than 780 nm.

While the invention has been described in detail and 55 with reference to specific embodiments thereof, it will be apparent to one skilled in the art that various changes and modifications can be made therein without departing from the spirit and scope thereof.

What is claimed is:

1. An electrophotoconductor for use in electrophotography, which comprises an electrically conductive support and a light-sensitive layer comprising a titanyl phthalocyanine dispersed in a binder and having the structure represented by the formula:



wherein  $X_1$ ,  $X_2$ ,  $X_3$  and  $X_4$  each and independently represent c or Br; and  $k$ ,  $l$ ,  $m$  and  $n$  each and independently represent zero or an integer of 1 to 4 and having the alpha-type crystallographic form.

2. An electrophotoconductor according to claim 1, wherein said alpha-type titanyl phthalocyanine, upon X-ray diffraction with Cu-K $\alpha$  radiation, provides characteristic peaks at Bragg angles ( $2\theta$ ) of 7.6, 10.2, 12.6, 13.2, 15.1, 16.2, 17.2, 18.3, 22.5, 24.2, 25.3, 28.6, 29.3 and 31.5.

3. An electrophotoconductor according to claim 1, wherein said light-sensitive layer is a single layer.

4. An electrophotoconductor according to claim 3, wherein said light-sensitive layer contains a charge transport material.

5. An electrophotoconductor according to claim 3, wherein said light-sensitive layer contains a charge generation material.

6. An electrophotoconductor according to claim 3, wherein said light-sensitive layer contains both a charge transport material and a charge generation material.

7. An electrophotoconductor according to claim 4, wherein said charge transport material is at least one compound selected from the group consisting of indoline compounds, quinoline compounds and triphenylamine compounds.

8. An electrophotoconductor according to claim 5, wherein said charge generation material is selected from the group consisting of perylene compounds and bisazo compounds.

9. An electrophotoconductor according to claim 7, wherein said indoline compound is represented by the formula:



wherein  $R_1$  is selected from the group consisting of alkyl, aralkyl, substituted aralkyl, aryl and substituted aryl;  $R_2$  and  $R_3$  are each independently selected from the group consisting of hydrogen, halogen, alkyl, aralkyl, substituted aralkyl, aryl and substituted aryl;  $R_4$  is

selected from the group consisting of hydrogen, halogen, alkyl, aralkyl and substituted aralkyl; R<sub>5</sub> and R<sub>6</sub> are each independently selected from the group consisting of alkyl, aralkyl, substituted aralkyl, aryl and substituted aryl and R<sub>5</sub> and R<sub>6</sub> may be bonded to each other to form a ring.

10. An electrophotoconductor according to claim 7, wherein said indoline compound is represented by the formula:



wherein A' is selected from the group consisting of aromatic hydrocarbon, substituted aromatic hydrocarbon, aromatic heterocyclic and substituted aromatic heterocyclic; and R<sub>1</sub>' and R<sub>2</sub>' are each independently selected from the group consisting of hydrogen, halogen, alkyl, aralkyl, substituted aralkyl, aryl and substituted aryl.

11. An electrophotoconductor according to claim 7, wherein said quinoline compound is represented by the formula:



wherein B' is selected from the group consisting of aromatic hydrocarbon, substituted aromatic hydrocarbon, aromatic heterocyclic and substituted aromatic heterocyclic; R<sub>1</sub>'' and R<sub>2</sub>'' are each independently selected from the group consisting of hydrogen, halogen, alkyl, aralkyl, substituted aralkyl, aryl and substituted aryl.

12. An electrophotoconductor according to claim 7, wherein said triphenylamine compound is represented by the formula:



5

wherein Ar<sub>1</sub>, Ar<sub>2</sub> and Ar<sub>3</sub> are each independently selected from the group consisting of aromatic hydrocarbon, selected aromatic hydrocarbon, aromatic heterocyclic and substituted aromatic heterocyclic.

13. An electrophotoconductor according to claim 8, wherein said perylene compound is represented by the formula:

15



20 25 wherein R<sub>1</sub>''' and R<sub>2</sub>''' are each independently selected from the group consisting of hydrogen, alkyl, aryl, substituted aryl and amino.

14. An electrophotoconductor according to claim 8, wherein said perylene compound is represented by the formula:



40

35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 998



(wherein — A'' — is a divalent conjugate organic group).

17. An electrophotoconductor according to claim 8, wherein said bisazo compound is represented by the formula:



(wherein — A'' — is a divalent conjugate organic group; and — B'' — is a monovalent organic group).

18. An electrophotoconductor according to claim 1, wherein said light-sensitive layer is a multi-layer which comprises a charge generation layer and a charge transport layer.

19. An electrophotoconductor according to claim 18, wherein said charge transport layer contains a charge transport material.

20. An electrophotoconductor according to claim 18, wherein said charge generation layer contains a charge generation material.

21. An electrophotoconductor according to claim 19, wherein said charge transport material is at least one compound selected from the group consisting of indoline compounds, quinoline compounds and triphenylamine compounds.

22. An electrophotoconductor according to claim 20, wherein said charge generation material is selected from the group consisting of perylene compounds and bisazo compounds.

23. An electrophotoconductor according to claim 21, wherein said indoline compound is represented by the formula



wherein R<sub>1</sub> is selected from the group consisting of hydrogen, alkyl, aralkyl, aryl and substituted aryl; R<sub>2</sub> and R<sub>3</sub> are each independently selected from the group consisting of hydrogen, halogen, alkyl, aralkyl, substituted aralkyl, aryl and substituted aryl; R<sub>4</sub> is selected from the group consisting of hydrogen, halogen, alkyl, aralkyl and substituted aralkyl; R<sub>5</sub> and R<sub>6</sub> are each independently selected from the group consisting of alkyl, aralkyl, substituted aralkyl, aryl and substituted aryl, and R<sub>5</sub> and R<sub>6</sub> may be bonded to each other to form a ring.

24. An electrophotoconductor according to claim 21, wherein said indoline compound is represented by the formula:



wherein A is selected from the group consisting of aromatic hydrocarbon, substituted aromatic hydrocarbon, aromatic heterocyclic and substituted aromatic heterocyclic; and R<sub>1'</sub> and R<sub>2'</sub> are each independently selected from the group consisting of hydrogen, halogen, alkyl, aralkyl, substituted aralkyl, aryl and substituted aryl.

25. An electrophotoconductor according to claim 21, wherein said quinoline compound is represented by the formula:



wherein B is selected from the group consisting of aromatic hydrocarbon, substituted aromatic hydrocarbon, aromatic heterocyclic and substituted aromatic heterocyclic; R<sub>1''</sub>, R<sub>2''</sub> and R<sub>3''</sub> are each independently selected from the group consisting of hydrogen, halogen, alkyl, aralkyl, substituted aralkyl, aryl and substituted aryl.

26. An electrophotoconductor according to claim 21, wherein said triphenylamine compound is represented by the formula:



wherein Ar<sub>1</sub>, Ar<sub>2</sub> and Ar<sub>3</sub> are each independently selected from the group consisting of aromatic hydrocarbon, substituted aromatic hydrocarbon, aromatic heterocyclic and substituted aromatic heterocyclic.

27. An electrophotoconductor according to claim 22, wherein said perylene compound is represented by the formula:



wherein R<sub>1</sub>''' and R<sub>2</sub>''' is each independently selected from the group consisting of hydrogen, alkyl, aryl, substituted aryl, and amino.

28. An electrophotoconductor according to claim 22, wherein said perylene compound is represented by the formula:



29. An electrophotoconductor according to claim 22, wherein said bisazo compound is represented by the formula:

wherein — A'' — is a divalent conjugated organic group; and — B'' — is a monovalent organic group.

30. An electrophotoconductor according to claim 22, wherein said bisazo compound is represented by the formula:



wherein — A'' — is a divalent conjugate organic group.

31. An electrophotoconductor according to claim 22, wherein said bisazo compound is represented by the formula:



— A'' — is a divalent conjugate organic group; and  
— B'' — is a monovalent organic group.

\* \* \* \* \*

